

# UNITED STATES PATENT OFFICE.

GEORGE H. RUPLEY, OF SCHENECTADY, NEW YORK, ASSIGNOR TO GENERAL ELECTRIC COMPANY, A CORPORATION OF NEW YORK.

## PROCESS OF INSULATING ELECTRICAL CONDUCTORS.

No. 835,827.

Specification of Letters Patent.

Patented Nov. 6, 1906.

Application filed January 13, 1906. Serial No. 295,868.

*To all whom it may concern:*

Be it known that I, GEORGE H. RUPLEY, a citizen of the United States, residing at Schenectady, in the county of Schenectady and State of New York, have invented certain new and useful Improvements in the Process of Insulating Electrical Conductors, of which the following is a specification.

This invention relates to the insulation of metal employed in electrical appliances, and finds special application in insulating wire, but is also used in other connections—such, for instance, as coating the core laminations of transformers. The process forms on the surface of the wire or other conductor a thin tough elastic firmly-adherent film which is waterproof, has high dielectric properties, is infusible at all temperatures to which it is exposed in service, is not inflammable, does not flow under pressure, and does not crack or scale off when the wire is bent even on a curve of small radius. Moreover, it is so thin as to enable a given length of wire to be coiled in considerable less space than is possible with cotton or silk covered wire.

This invention constitutes an improvement on that set forth in my previous patent, No. 806,574, granted December 5, 1905. The process therein disclosed is entirely successful in practice; but it has been found that by modifying my process as hereinafter set forth an insulation is obtained which is more desirable for certain classes of work.

The process as heretofore carried on and as set forth in the above-mentioned patent consists of previously thickening a quantity of vegetable oil, such as linseed-oil, by the application of heat, dissolving the residuum in a suitable solvent, supplying a film of the solution to the conductor, and hardening the coating by the application of heat. As set forth in my previous patent, the thickening is accomplished by mixing a suitable quantity of commercial linseed-oil with a certain percentage—say of two per cent.—of oxid of zinc and a substantially similar quantity of oxid of lead. The mixed mass is then raised to a temperature of from 550° to 600° Fahrenheit and the heat continued until the oxid is entirely taken up by the oil and the required degree of distillation effected during which the glycerids are broken up and glycerin set free. When the mass acquires a good degree of stiffness, about twenty-five per cent. of a

refractory solvent, such as rosin-oil, is added and the mass allowed to cool. The film is then hardened by the application of heat, and the arrangement whereby it is accomplished is fully set forth in the above-mentioned patent. The result of this process is a smooth, black, and glossy coating of a residuum of the oil. It has been found, however, that for certain uses it is preferable to have an insulation which does not have a gloss or polish, but which will have a dull finish slightly roughened, so that there will be more friction between the turns. This is found particularly desirable in certain kinds of winding—as, for instance, in the case of universal winding, where it is essential that there be more surface friction than in other methods of winding. For these reasons and also to give body to the insulation and to form a mechanical separator I add a certain amount—say from five to ten per cent.—of some solid material, such as china-clay or lump clay. Other powdered or granulated neutral or inert materials may of course be substituted without departing from the spirit of my invention and the percentage will likewise be varied. This material is preferably added after the residuum has been thinned down by means of the solvent. It is possible by this process to obtain a thicker insulation with a less number of applications, which in some instances is desirable, especially in the case of plates or large wire, where considerable pressure may be applied to the conductor. The dull finish given to the wire also has advantages which will be evident to those skilled in the art. The inert filler is also of special advantage where great pressure is used, as it acts as a resisting spacer.

While I have described my invention as consisting of certain steps in the process and in the use of certain materials, it should be understood that I do not limit my invention to the particular materials or process steps except as it is limited by the scope of the claims annexed hereto.

What I claim as new, and desire to secure by Letters Patent of the United States, is—

1. The process of insulating an electrical conductor which consists in substantially freeing an oil from the glycerin of combination mixing a powdered material with the resultant product, applying a film of the mix-

ture to the conductor, and hardening the film by heat.

2. The process of insulating an electrical conductor which consists in substantially freeing linseed-oil from the glycerin of combination mixing a powdered material with the resultant product, applying a film of the mixture to the conductor, and hardening the film by heat.

3. The process of insulating an electrical conductor consisting in dissolving a previously-thickened and partially-decomposed oil in a suitable solvent, mixing a quantity of solid matter with the solution, applying a film of the solution to the conductor, and hardening the film by heat.

4. The process of insulating an electrical conductor consisting in mixing a quantity of powdered material with a vegetable oil substantially free from glycerin, applying a film of the compound to the conductor, and hardening the film by heat.

5. The process of insulating an electrical conductor which consists in setting free the glycerin and fatty acids in a quantity of linseed-oil, driving off the glycerin, mixing a quantity of granular material with the fatty acids, applying a film of the mixture to the conductor, and then hardening the film by heat.

6. The process of insulating an electrical

conductor consisting in substantially freeing a quantity of vegetable oil from glycerin, mixing a heat-refractory powder with the resulting product, applying a film of the mixture to the conductor, and then hardening the coating by heat.

7. The process of insulating an electrical conductor consisting in mixing one or more metallic oxids with a vegetable oil, boiling the mixture to break up the glycerids and free and drive off the glycerin, dissolving the residuum in a suitable solvent, mixing a quantity of silicate with the solution, applying a film of the resulting mixture to the conductor, and hardening the film by heat.

8. The process of insulating an electrical conductor consisting in mixing one or more metallic oxids with linseed-oil, maintaining the mixture at a temperature above 500° Fahrenheit until it becomes stiff and elastic at ordinary temperatures, dissolving the stiffened mass in a refractory solvent, mixing a quantity of clay with the solution, and hardening the coating by heat.

In witness whereof I have hereunto set my hand this 11th day of January, 1906.

GEORGE H. RUPLEY.

Witnesses:

BENJAMIN B. HULL,  
HELEN ORFORD.